

## UNITED STATES PATENT OFFICE.

HENRY GARDNER, OF DETROIT, MICHIGAN, ASSIGNOR TO FORD MOTOR COMPANY, OF HIGHLAND PARK, MICHIGAN, A CORPORATION OF DELAWARE.

## PLATING AND METHOD OF ACCOMPLISHING THE SAME.

No Drawing.

Application filed February 19, 1923. Serial No. 620,040.

In the process of producing a finished nickel plated article there are numerous operations incurring time, labor and expense, and one of these operations is that of buffing or polishing the nickel plated article by using some polishing material which will impart lustre, "color" or a high degree of finish on the article. This last mentioned operation materially lessens the durability of the article, particularly if the article possesses corners or edges which are subjected to wear.

My invention aims to simplify the process of producing a finished nickel plated article by eliminating the operation referred to above, whereby the following advantages are gained.

First, besides eliminating the time, cost and labor incident to the buffing or polishing operation, I obtain an article or plate of uniform thickness, particularly at its corners or edges thus insuring greater wear.

Second, the finish and texture of the coating on the article are materially improved, without any danger of "peeling" or cracking of the nickel coating.

My invention further aims to improve the process of nickel plating by using a nickel plating solution or bath which, during the process of nickel plating, will prevent pitting of the article or plate being treated and insure a final finish possessing a desired degree of lustre or color. The advantages gained by my improved nickel plating bath or solution may be characterized in the following particulars.

First, the time in which articles are immersed in the nickel plating solution is materially reduced, approximately one-half, thus insuring a greater production of nickel plated articles or plates.

Second, the bath or solution can be easily and quickly changed to produce an article or plate having a desired degree of finish or lustre ranging from dullness to brightness, consequently the bath or solution being used to produce one grade of articles can be quickly changed to produce another grade of articles without discarding or wasting the initial bath or solution.

Third, the improvement entering into the

bath or solution is applicable to other plating processes than that of nickel plating, and as an instance of other plating I may mention copper plating for the reason that the finish imparted to copper insures an indurate coating having a high degree of lustre.

It is by virtue of the improved plating bath or solution that I gain the first mentioned advantages, namely that of eliminating the buffing or polishing operation and by producing an article equally as good, if not better, with a proportionate increase in the production of such articles.

In order that my improvement may be more fully understood, I will briefly consider nickel plating as an instance of a plating process in which my improvement has been successfully used and produced good results. In an ordinary nickel plating process, the article to be plated is thoroughly clean. This may be accomplished by a series of dipping in suitable chemical solutions rinsing waters, and subjecting the article to an electrolysis action in chemical baths, so that the article is chemically clean for plating purposes.

Should the article to be nickel plated be of a ferrous nature it is customary to first copper plate the article by immersing it in a copper solution in an electro-plating tank, for a period of time necessary to deposit the proper coating of desired thickness. Following either the copper plating operation or the cleaning of the article for the nickel plating operation, the article must be burnished or buffed on the surface to be nickel plated, and the extent of burnishing or buffing depends upon the smoothness of the final finish to be imparted to the article.

With the article prepared in either of the above recited ways, it is now ready to be immersed in a nickel plating bath or solution. As an instance of such bath I may mention as added to each gallon of water sulphate nickel salts, single or double 12 ounces, and boracic or muriatic acids 4 ounces;—or ammoniacal solution of ammonium-nickel sulphate receiving a nickel anode, while the article is the cathode in circuit with a suitable source of electrical

energy affording from one to five volts according to the amount and surface to be nickel plated.

To each hundred gallons of either of the above baths or solutions I add

|                              |            |
|------------------------------|------------|
| Cadmium chloride or sulphate | 81         |
| Glycerine                    | 200 to 800 |
| Lead sulphate                | .266       |
| Lead carbonate               | "          |
| Or lead monoxide "litharge"  | "          |

The composition of the solution matter or bath may be varied somewhat in each particular so that there may be various bath formulas for nickel plating purposes. For instance, to one gallon of water there may be the following admixture:

|                                |                |
|--------------------------------|----------------|
| Sulphate nickel salts (double) | 8 oz.          |
| Sulphate nickel salts (single) | 4 "            |
| Boracic acid                   | 2 "            |
| Muriatic acid                  | 1/4 "          |
| Cadmium chloride               | 3 pennyweights |
| Glycerine                      | 1/2 oz.        |

Then again, I may dispense with the lead compounds or cadmium and simply depend upon glycerine to obtain a similar result. I may also substitute molasses for the glycerine in either of the above combinations.

As is the usual practice, the article to be plated is suspended in the solution or bath for a period of time necessary to furnish the article with a coating of desired thickness, and in addition to the time element the current voltage, the amperage used, and the strength of the solution determine to a certain extent the final result. For a heavy coating or a large amount of material the time of immersion is proportionately lengthened, and whatever the time may be the article is allowed to remain in the solution until it becomes bright and has a high lustre, when it is removed from the solution, rinsed in cold water, subjected to an acid bath, and again rinsed and which will permit the article to be eventually dry without being spotted and at the same time preserve the finishing color imparted to it.

I find that cadmium in a nickel plating bath or solution tends to reduce the size of the grains of the nickel and that this action is further increased by the addition of glycerine. Either of these ingredients, in a suitable carrying agent, will enhance the final appearance of the article by eliminat-

ing pitting and producing an exceedingly bright surface.

It is thought unnecessary to set forth the various chemical actions which may take place during the electrolysis action, and I would have it understood that my invention, in its broadest aspect, involves the use of modifying addition to the plating bath of cadmium, glycerine or any equivalents or combinations thereof that will cause a coated article to be produced, by electroplating, which does not require a final buffing or polishing operation.

What I claim is:-

1. A solution for a nickel plating tank comprising the following ingredients in the proportions set forth: water one gallon, sulphate nickel salts (double) 5 to 12 ounces, sulphate nickel salts (single) 1 to 8 ounces, boracic acid 1/2 to 4 ounces, muriatic acid 1/8 to 3/4 ounces, cadmium chloride 1 to 8 pennyweights, and glycerine 1/8 to 1 ounce.

2. A solution for a nickel plating tank comprising the following ingredients in the proportions set forth: water, one gallon; sulphate nickel salts (double) 8 ounces, sulphate nickel salts (single) 4 ounces, boracic acid 2 ounces, muriatic acid 1/4 ounce, cadmium chloride 3 pennyweights, and of glycerine 1/2 ounce.

3. In a nickel plate solution the combination of a solution of nickel salts of a strength suitable for plating purposes with a small percentage of cadmium salts and a suitable carrying agent.

4. In a nickel plate solution the combination with nickel salts in solution of glycerine with a small percentage of cadmium salts as a means of producing a lustrous coating on an article plated thereby.

5. A solution for a nickel plating tank comprising the following ingredients in the proportions set forth, to one gallon of water, add from 5 to 12 ounces of nickel ammonium sulphate, 1 to 8 ounces nickel sulphate, 1/2 to 4 ounces boracic acid, 3/2 ounce sal-ammoniac, 1 to 8 pennyweights cadmium chloride, 1/8 to 2 ounces glycerine.

6. A solution for a nickel plating tank comprising the following ingredients in the proportions set forth, to one gallon of water, add 8 ounces of nickel ammonium sulphate, 4 ounces nickel sulphate, 2 ounces boracic acid, 3/2 ounce sal-ammoniac, 3 pennyweights cadmium chloride, 1 1/2 ounces glycerine.

In testimony whereof I affix my signature.

HENRY GARDNER.